

## UNITED STATES PATENT OFFICE

1,940,486

GLUE PRODUCT AND METHOD FOR  
PREPARING THE SAME

Charles H. Campbell, Kent, Ohio

No Drawing. Application May 22, 1933  
Serial No. 672,343

9 Claims. (Cl. 134—46)

This invention relates to a glue product and to a method for preparing the same.

Heretofore high grade glues have been used in coating compositions such as calcimine and similar coating compositions in which the vehicle is water. The high grade glue used for this purpose will go into solution in water only with great difficulty and only by heating the water to temperatures from 140° to 160° F. Glues have 10 been chemically treated in various ways to make them more readily soluble in water but such treatments of the glue affect the adhesive qualities thereof.

The general purpose of the present invention 15 is to provide an improved glue product and method for making the same whereby the physical properties of the natural glue are substantially unaffected and yet the glue will be readily soluble in water at ordinary atmospheric temperatures and even temperatures as low as 40° F.

In particular the invention has for its object 20 the application of glue in very thin or microscopic films over a base of finely divided, preferably inert, material or such material in a colloidal state such as whiting, gypsum or other materials so that the thin films of glue on these base materials are readily acted upon by water, causing the glue to jell readily and to go into 25 solution at ordinary temperatures and even temperatures as low as 40° F.

It is a further object of the invention to provide a simple, effective procedure for making the above-described product economically by the elimination of a number of steps in the usual 30 process of manufacturing glue compositions.

The foregoing and other purposes of the invention are attained in the material and by the method set forth in the succeeding paragraphs hereof. It is to be understood that the invention 35 is not limited to the specific form thereof described.

Animal glue is a colloid and is affected by heat and moisture, especially by long-continued heat, and long, low heats with moisture are more 40 harmful than higher heats for a short time. On this account glue and gelatin manufacturers spread the chilled sheets as thin as possible in drying on nets to prevent loss of strength. By this method the moisture lifts much more easily 45 in a shorter time.

In accordance with one prior practice, some calcimine manufacturers have taken glue and the other bases commonly used in this manufacture and after dissolving the glue mixed it 50 with the bases desired, making a thin paste or

magma, and dried the same on pans in dry kilns. The objection to this method was that the glue and other bases separated in the drying, the glue floating to the top of the pan, and in the subsequent grinding a large part of the glue was ground separately. If the manufacturer started with a high grade glue, he found after this operation the glue had lost from twenty-five percent to thirty-five percent of its original strength, depending upon the time of heating 60 and the temperature employed. Moreover, he had not been able to really coat his bases with the glue. The microscope revealed that a portion of the particles of base used had particles of glue adhering to them by only a point; the balance of the glue was present only in the form of a mixture. When glue is in calcimine as a simple mix there is always a tendency of the particles to agglomerate and roll into balls when water is added, but when fine base particles are 65 really coated with very fine films of glue this tendency is not present.

Other manufacturers at a somewhat later period utilized a method whereby the glue was dissolved and mixed with the bases in a mixer 70 until thoroughly incorporated, adding just enough water to make a mix possible. This magma was then taken and placed in a rotary dryer with mixing arms to prevent the magma from separating during the drying operation. In using 75 this process, which is the commercial process now, a comparatively high heat is maintained so as to reduce the time the glue is under heat. This process reduces the test of the glue fifteen to twenty-five percent, depending upon the time 80 and temperature of the heat treatment. The particles of base agglomerate and the dried material rolls from the dryer with many lumps. These lumps are quite hard, being cemented together by the glue and are ground with difficulty. 85 This accounts for the fact a calcimine of this description does not take the water well and it is usually necessary to strain before using. In fact, straining is a recognized procedure. As shown by the microscope, about one-half the 90 glue in such calcimine is present in glue particles merely mixed with the other materials and difficult to dissolve and that adhesively attached particles are more or less only in the form of partial attachment of particles and not a real coating.

The ability of any calcimine to cover a given wall surface per pound of calcimine used depends upon the particle size of the whiting or other base used. The smaller the particle size 95

of the base the greater the covering quality. Some manufacturers, although using good grades of whiting, obtain poor results due to the coarse grinding.

5 While many attempts have been made to produce a commercially feasible, cold water soluble calcimine with high grade glue, a cold water soluble calcimine has heretofore been made only by using soluble starches or low grade glues instead of high grade animal glue. A calcimine of this sort will not second coat but pulls if the operator tries to retouch due to defective covering in the first case. Many times an entire wall must be washed and redecorated. The calcimines in general use are simple mixtures using a high grade glue as the adhesive, and requiring the use of hot water in the mixing to dissolve the glue. A high grade glue resists the absorption of water, takes time to jell before going into solution, and requires heat. But high grade glue, while difficult to put into solution, resists the action of water and the brush in second coating. Practically all hot water calcimines today will take a second coat because all contain good grades 25 of glue. But all require hot water, and time. In new buildings the practice is to put the calcimine into solution at night so as to avoid the delay during the day incident to the making of the solution and straining preliminary to application.

30 In accordance with this invention a high grade glue is used that under ordinary usage could not be put into solution in anything but hot water. This glue in solution has a particle size and the jell strength and viscosity are due to particle size. Very high temperatures applied to such glues for a short time do less injury to the glue colloid than any other form of drying and the glue retains its physical qualities better and its properties of adhesion are not substantially damaged. The brushing quality of a calcimine depends upon the viscosity of the glue used. It is desirable that a calcimine when applied pull a bit on the brush, this insuring a good even spread. It accordingly will be understood why hot water 45 grades have heretofore been the rule.

By first running a good grade of whiting through a colloid mill the number of particles per pound are increased and the covering quality of the finished calcimine is improved. Not all 50 of the whiting will be reduced to colloid size so as to show a true Brownian movement under the microscope, but the particle size is reduced to a finer state of sub-division than possible by any ordinary milling used today. A whiting ground 55 as above will have a twenty percent better covering quality than ordinary ground whiting.

By taking then a very finely divided whiting and mixing it with a thin solution of high grade glue in the proportion of about one part of dry 60 glue in solution to three to eight parts of whiting used with enough water added to make the finished magma about twenty percent solids and then flash drying, a cold water soluble calcimine containing a high grade glue is obtained with 65 the natural qualities of the glue unharmed. The resulting material consists of a very finely divided base material, each particle of which is coated with a thin glue film so finely divided that even a high grade glue will go into solution in water at 40° F. If for any reason very low temperatures 70 are desired for the finished calcimine the percentage of base is increased, thereby reducing the film of glue on the whiting particles. A study of this material under the microscope shows not just the ordinary mix with some attachment of 75

particles, but a real coating of very fine base particles with a high grade glue that because of its exceedingly fine film size is actually soluble in cold water as low as 40° F. Ten percent or less of the glue is present as a mere mixture and this has a thin, flaky form.

80 A high grade hide glue such as used in hot water calcimine is made from hide scrap and after cleansing, washing and bleaching goes to the glue kettles and the glue is boiled out of the stock. After this the glue liquor is settled, filtered, chilled, cut into sheets, spread on nets, dried, removed from the nets, ground, and finally packed. The drying of the glue in the thin, transparent sheet of commerce is a part of the 85 glue cycle in producing glue. In carrying out this invention it is preferred to take the glue fresh from the kettles and mix with it immediately the finely divided base and flash dry as stated without injury to the physical properties 90 of the glue. As finished dry glue may be used by preparing a thin, hot solution, but a thin, hot solution direct from the glue kettle appears to give the best results in that it gives a thinner coating of the base particles and, moreover, by 95 using the glue direct from the kettles the balance 100 of the steps in the usual manufacture of the glue is eliminated.

It is not known with certainty why there is loss of strength of glue in ordinary drying when 105 the glue is exposed to the action of heat and moisture over a period of time. Some say the action of heat and moisture splits the particle size, and others the effect of oxygen in the heated currents of air used in drying, and some say 110 both. By drying in the presence of an inert gas such as carbon dioxide, the present inventor has found that the drying may be accomplished with less damage to the glue. An atmosphere of CO<sub>2</sub> gas in whole or in part may be used instead 115 of air. However satisfactory results are secured using only air.

120 In carrying out the invention in its preferred form, liquid glue such as produced by extraction from tanner hide scrap or bone prior to the usual step of evaporation has mixed therewith 125 whiting, gypsum, or other suitable mineral or other bases, either finely ground or in a colloidal state. The whiting or gypsum may be first passed through a colloid mill. However, the invention may be carried out with these materials in a finely ground or pulverous state. The proportions of the ingredients in the batch thus made may be

1 part (solid content) \_\_\_\_\_ glue 130  
3 to 5 parts \_\_\_\_\_ whiting  
12 to 20 parts \_\_\_\_\_ water.

135 This usually requires that the liquid glue extracted from the tanner hide scrap or bone shall be somewhat diluted either before or after the addition of the whiting or gypsum.

140 The batch thus made is then dried in such a way as to prevent agglomeration of the finely ground or colloidal particles of base material. This may be accomplished by flash or spray drying, i. e., the batch may be sprayed by any suitable means in a more or less nebular state into a hot atmosphere or against a hot surface such as the surface of a heated drum from which the material may be scraped by a doctor blade. The material will be quickly dried with no appreciable effect upon the adhesive properties of the glue. This is preferably accomplished in an atmosphere principally of CO<sub>2</sub> with or without 145

some air at a high temperature, for example 500° to 600° F. This will accomplish the drying in a period of from one-fourth to one-third of a second and with no appreciable oxidation of the glue. The material thus produced is preferably quickly cooled after the drying to avoid oxidation.

The flash or spray drying may be accomplished by the use of suitable equipment resistant to abrasive action of the base materials. A diamond set nozzle may be employed for this purpose in which case the pump pressure on the liquid batch will be from 2,000 to 3,000 pounds per square inch to produce a nebular spray in which there is no appreciable tendency for the particles to agglomerate. Instead of the diamond set nozzle, a centrifugal disc spraying device may be employed. The disc in this device, from which the material is thrown in a spray, should be revolved at a rate of from 9,000 to 10,000 R. P. M. to obtain the best results and produce the finest possible state of particle subdivisions. At any rate the forces tending to disperse the glue must be sufficient to overcome the cohesion of the glue particles, otherwise lumps comprising a spongy mass of agglomerated particles are produced. In spray drying it is very necessary to prevent sponging in drying. Some types of spray dryers are impossible because this feature cannot be prevented with their usage.

The resulting material comprises fine particles of whiting or other mineral base with each particle coated with an exceedingly thin or microscopic film of glue along with a small percentage of flaky glue particles. This glue, because of the extreme thinness of the films, is readily jelled by water and readily goes into solution therein at low temperatures.

The process may be varied by the addition of such other materials to the batch as may be desired. For example, in the production of a calcimine all the ingredients of the calcimine might be mixed in the glue and glue base solution and flash-dried therewith under the conditions prescribed. However, it is usually preferable from the standpoint of economy and handling of materials to mix the balance of the ingredients of the calcimine to the glue and glue base product after the latter has been prepared as described.

Modifications of the invention may be resorted to without departing from the spirit thereof or the scope of the appended claims.

What is claimed is:

1. That method for making a glue product which comprises mixing with liquid glue a finely powdered, inert base, flash or spray drying the mixture in a heated atmosphere including a large proportion of an inert gas, and quickly cooling the material thus produced whereby non-agglomerated particles of the base are produced which are coated with films of glue readily soluble in cold water.

2. That method for making a glue product which comprises mixing a finely powdered, inert base with a thin solution of glue in water and spray-drying the mix to form non-agglomerated

particles of the base with thin films of glue thereon which are readily soluble in cold water.

3. That method for making a glue product which comprises mixing with a solution of glue and water a finely powdered whiting, and flash-drying the mix in an atmosphere principally of CO<sub>2</sub>.

4. That method for making a glue product which comprises mixing with a solution of glue and water a powdered whiting, and flash-drying the mix to form non-agglomerated particles of the base with thin films of glue thereon which are readily soluble in cold water.

5. That method for making a glue product which comprises mixing directly with the solution of animal glue formed by extraction in the usual way, a finely ground mineral base, and spray-drying the mix in a nebular state in an atmosphere at a high temperature whereby the particles of said mineral base do not agglomerate and are coated with thin films of glue readily soluble in cold water.

6. That method for making a glue product which comprises mixing finely ground particles of a base with a thin solution of glue, and spray-drying the mix in a nebular state in an atmosphere at a high temperature to produce non-agglomerated particles of the base coated with films of glue readily soluble in cold water.

7. A spray or flash-dried product of manufacture for use in calcimine and like coating compositions, said product comprising whiting of about colloidal size, the particles of which are coated with a microscopic film of extracted animal glue of a type which normally is not soluble in cold water, the films of glue on said particles being so thin as to be readily soluble in cold water, said glue being substantially of the strength, jell and viscosity of the glue as originally extracted.

8. A spray or flash-dried product of manufacture for use in calcimine and like coating compositions utilizing water as the vehicle thereof, said product comprising filler particles inert to glue and water and of about colloidal size, said particles being coated with microscopic films of extracted animal glue of such thinness as to be readily soluble in cold water, said glue being normally of a type which is insoluble in cold water said glue having substantially the chemical composition, strength, jell and viscosity of said glue in its original extracted condition.

9. A spray or flash-dried product of manufacture for use in calcimine and like coating compositions in which water is the vehicle comprising non-agglomerated particles of a filler inert to glue and water having thereon microscopic films of extracted animal glue of a type which will not normally dissolve in cold water, said films being so thin as to be readily soluble in cold water, said glue having substantially its original strength and viscosity when dissolved and being of substantially its original chemical composition as obtained when said glue was originally extracted.

CHARLES H. CAMPBELL.